

## UNITED STATES PATENT OFFICE

CARLETON ELLIS, OF MONTCLAIR, NEW JERSEY, ASSIGNOR TO ELLIS-FOSTER COMPANY, A CORPORATION OF NEW JERSEY

## GREASE-RESISTING BOX BOARD

No Drawing. Application filed August 22, 1927. Serial No. 214,781.

This invention relates to grease-proof paper or paper which is relatively resistant to penetration by greasy substances and to the process of making same, and the invention also includes as an article of manufacture containers made from such grease-resistant paper.

In using the term "paper" herein, I embrace not only the thinner grades of paper, but also the heavier grades, particularly those designated as board stock.

The present invention enables thin grease-resistant paper to be made which in itself is not sufficiently thick or rigid to be self-supporting, but may be employed as a lining for containers made of stiffer material. On the other hand by treating paper board in the manner described herein, I am enabled to secure a sheet which has sufficient strength and 20 rigidity to be employed of itself in making boxes, cartons, ice cream containers, milk and other liquid containers, oyster pails and the like.

It is a great advantage in making boxes not 25 to be obliged to insert a special lining, and the preferred form of the present invention enables a grease-resistant container, such for example as a cracker, biscuit or caddy box, to be made without resort to a sheet of viscose 30 as a lining material.

The procedure set forth in the present invention is applicable to various grades of paper, but may be used to advantage with cheaper kinds of paper or board, particularly 35 those containing ground wood. Thus I am able to employ a mixture of ground wood and sulphite pulp and the like to make a board suitable for the purpose. I do not, however, limit myself to any particular grade or thickness 40 of paper and paper board.

The paper may be suitably sized if desired with rosin size or with wax emulsion, or with mixtures of rosin size and wax emulsion, or the paper, during formation, may be built 45 up of layers of pulp with intermediate layers of asphalt or other waterproofing emulsion and the like.

Preferably I employ a paper or board made from ground wood and sulphite pulp or similar fibrous material, containing wax which

has been added in the form of an emulsion in the beater.

In whichever way prepared the dry paper is coated preferably only on one side with a grease-resisting composition comprising a 55 compound of cellulose which is soluble in organic solvents, including nitrocellulose, cellulose acetate, and cellulose ethers.

The present invention will be described particularly with reference to the employment of 60 nitrocellulose. While high viscosity nitrocellulose such as smokeless powder, or celluloid cotton may be used in the composition employed, I prefer to utilize nitrocellulose of low viscosity. Thus on the one hand I may 65 employ the extremely low viscosity nitrocellulose ranging from one second, down to one-half second or even lower, or I may use intermediate low viscosity ranging from 1 or 2 seconds up to 4 or 5 seconds, or still higher 70 viscosities running from 5 to 15 seconds.

Smokeless powder which has become too old to be employed in military operations affords a cheap supply of nitrocellulose. It is, however, of such high viscosity that a 75 large amount of solvent would be required to form a solution which could be readily applied to the paper to produce the grease-resistant coating. Preferably, therefore, I employ smokeless powder of reduced viscosity. This may be obtained by heating the smokeless powder or by treating it in solution with ammonia or other alkali agents as is now known in the art.

Thus smokeless powder may be dissolved 80 in acetone and a small amount of ammonia gas allowed to pass into the solution. On standing for a few hours reduction in viscosity will take place, and any free ammonia may be suitably neutralized. Treatment 85 with chemical agents in this manner tends somewhat to discolor the nitrocellulose in some cases, unfitting the solution for use as a lacquer for certain purposes, but in the present invention the paper itself in its preferred form, that is one containing ground wood or its equivalent or other low grade paper raw material, does not yield a paper or board which is white in color, but one 90 which is yellowish or brownish.

As solvents for the nitrocellulose, I have preferred to employ highly volatile ones. The more expensive high boiling solvents, such as amyl acetate, butyl acetate, ethyl lactate and the like are costly, and while I propose to recover the solvents as far as possible, there is always some loss, and the solvent cost is thus considerably increased when more expensive solvents are used.

10 A solvent such as acetone has many advantages, one being that it forms probably the least viscous nitrocellulose solution of any common available solvent. It is obtainable in large quantities. Moreover, it is a strong solvent for resins and balsams, and other substances which may be added to the nitrocellulose to increase the content of total solids. A solution of nitrocellulose in acetone, when allowed to evaporate, becomes white and opaque, either not forming any film, or one of poor strength. This whitening or blushing of the film is highly objectionable in most coating compositions. It is not so important in connection with the present invention, but at the same time is a desirable condition to avoid since the weakening of the coating due to blushing, renders the coating more liable to crack on folding when the coated paper is formed into a box or carton. It is desirable to avoid any cracking at the creases.

15 In Serial No. 117,152, filed June 19, 1926, I have disclosed the use of a blush-corrective resin employed in a coating composition comprising nitrocellulose dissolved in a volatile vehicle of a blush-forming character, and with respect to certain phases of the present invention certain features disclosed in the aforesaid application are employed herein with reference to the grease-proofing of paper.

20 Unlike natural resins which have no such action on nitrocellulose and which merely mix with nitrocellulose in solution, certain types of synthetic resins have been found to possess a noticeable colloiding effect and great compatibility for nitrocellulose. Particularly is this true of those synthetic resins which can be made by chemically combining glycerol or other polyhydric alcohols with phthalic acid or its anhydride, or various modifications thereof. Other polybasic acids such as citric, tartaric, maleic, malic, and like substances, are, in most cases, suitable for similar purposes. In place of glycerol, I may employ such other polyhydric alcohols as ethylene and propylene glycols, mannitol, pentaerythritol, and like substances. Various mixtures of acids are often more desirable than any one acid. Thus resins made from phthalic anhydride and glycerol may be advantageously modified by incorporating certain amounts of the fatty acids of various oils such as cottonseed oil, linseed oil, and the like, or by means of monobasic carboxylic

acids, such as benzoic, salicylic, benzoyl-benzoic acid, and the like.

One suitable resin, for example, is made substantially as follows:

25 47 parts by weight of glycerol are added to 80 parts by weight of phthalic anhydride and 40 parts by weight of the distilled fatty acids obtained from cottonseed oil. The mixture is heated in a suitable container such as an aluminum kettle, preferably closed at the top, except for an air-cooled reflux condenser, and the mixture is heated slowly, preferably with mechanical agitation, to a temperature of about 280° C. until a sample of the mixture has shown the desired hardness or the acidity 80 has been sufficiently reduced, e. g., so as to have an acid number of substantially less than twenty. Another suitable resin is made from glycerol 47 parts by weight, phthalic anhydride 118 parts by weight, and benzoic acid 98 parts by weight. This resin is made in identical manner as the foregoing resin.

85 Still another suitable resin of a harder nature may be made by combining 47 parts by weight of glycerol with 94 parts by weight of phthalic anhydride. This mixture is inclined to polymerize and become infusible at higher temperatures, or if heated for too long a period, so that it is advisable to heat this mixture to a temperature not substantially in excess of 230° C., and continuing until a sample has shown the desired degree of hardness.

90 These synthetic resins are soluble in acetone and many other solvents and may be incorporated with nitrocellulose in any desired proportion to form suitable coatings. It is usually necessary to employ a fairly large proportion of these resins, for example, at least equal parts of resins and nitrocellulose 100 and preferably somewhat more, in order to obtain the desired effect. Plasticizers or softeners for nitrocellulose may be added where desired, such materials as diethyl or dibutyl phthalate and tricresyl phosphate 105 being especially recommended.

110 These synthetic resins with nitrocellulose, with or without plasticizers, pigments, dyes, or other substances, may be dissolved in acetone, ethyl acetate, mixtures thereof, with or without the addition of diluents such as low boiling alcohols, benzol, and the like, to form solutions of suitable characteristics. By means of these synthetic resins I am able to use these low boiling solvents with nitrocellulose and obtain clear and transparent and non-blushing films at ordinary room temperature. This effect cannot be obtained from natural resins such as rosin, rosin ester 115 and damar, or other resins which have no appreciable solvent action for the nitrocellulose.

120 One suitable composition may be made by dissolving one part by weight of one-half second viscosity nitrocellulose and 2 parts by 130

weight of a cottonseed fatty acid phthalic glyceride resins in 7 parts by weight of acetone. Other synthetic resins having for nitrocellulose the properties aforesaid, may 5 be employed in place of the one specified.

Esterified rosin such as rosin glyceride, or ordinary ester gum may be added to the above compositions, also the glycol esters of rosins, or the glycol-ether esters of rosin. Likewise 10 other resins and balsams may be introduced where such addition cheapens the composition without destroying its desirable properties.

The following will illustrate different compositions suitable for the coating operation:

#### Example I

Low viscosity nitrocellulose one part by weight was dissolved in acetone 4 parts, forming 20 a 20% solution.

Cottonseed phthalic glyceride resin was dissolved in an equal volume of acetone, thus making a 50% solution.

A paper coating composition was made by 25 mixing 8 parts by weight of the resin solution, with 20 parts of the nitrocellulose solution, adding one part of dibutyl phthalate.

The viscosity of this solution is quite low, and it may be applied to paper by brushing 30 or coating apparatus. It may be made of even higher consistency when applied with special coating means.

#### Example II

Low viscosity nitrocellulose was dissolved 35 in a mixture of equal volumes ethyl acetate and benzol to form a 20% solution.

Cottonseed phthalic glyceride resin was dissolved in a similar composite solvent to 40 make a 50% solution.

These were mixed in the same proportions as stated in Example I, including the addition of one part of dibutyl phthalate. The viscosity was considerably higher than that 45 of Example I, although the same grade of nitrocellulose was used in both cases. In order to obtain approximately the viscosity of Example I, the composition of Example II was diluted with 7 parts of a mixture of equal 50 parts ethyl acetate and benzol.

This was applied to paper and paper board and gave an excellent coating.

#### Example III

An alcohol-soluble nitrocellulose of  $\frac{1}{2}$ -second viscosity, one part, was dissolved in a mixture of denatured alcohol, 2 parts; ethyl acetate, one part; benzol, 2 parts.

Cottonseed phthalic glyceride resin was 55 dissolved in an equal weight of a mixture of equal parts denatured alcohol and benzol.

200 parts of the nitrocellulose solution were mixed with 66 parts of the resin solution and 10 parts of dibutyl phthalate.

65 80 parts of a mixture of equal volumes de-

natured alcohol and benzol were added. This composition was applied successfully to paper to form a grease-resisting coating.

The process of applying these solutions to the paper surface preferably consists in passing the web of paper through coating rolls to which the composition is fed, and immediately passing the coated paper into a drying oven, where at a gentle heat the highly volatile solvents evaporate quickly and are withdrawn by a pump to a solvent recovery apparatus. Since the paper preferably is coated only on one side, it is very readily handled in the coating apparatus, and on the carriers conveying to the drying chamber.

The final operation forming a feature of the preferred embodiment is that of hot calendering the coated surface. The grease-resisting qualities appear to be increased by hot calendering, and various slight blemishes, particularly iridescent spots or areas, are eliminated. The temperature of the calender rolls will vary depending on the composition employed for coating and the speed of travel of the web of paper through the rolls. Preferably, I allow just enough heat and time of contact to slightly soften the coated surface. By employing a synthetic resin or balsam having a mild solvent effect on the nitrocellulose at elevated temperatures, an improved grease-resisting effect results.

It should be noted that the coating thus applied does not need to be thick, but may be of such thinness that the finished paper or board shows scarcely any evidence of treatment, such very thin nearly invisible coatings after hot calendering serving to provide a sufficient grease-resistance, so that the resulting board may be made into cartons for crackers and other foods containing a considerable amount of shortening and not showing grease marks through the board, even though the crackers or biscuit may be in contact therewith for a long period of time.

The board thus may be treated with the grease-repellant resinated nitrocellulose to form a surface impregnum which scarcely increases the thickness of the paper. This thin surfacing of resinated nitrocellulose applied only to one side of the board enables paper to be folded into box shape with the surfacing, or surface impregnum, on the interior of the box only. The folding of the paper or board therefore does not stretch the surfacing, but contracts or compresses it, as the folding is, in most cases, inward on the side where the surfacing exists. Thereby a carton adapted as a package for fat-shortened food products, such as biscuit, crackers, and cookies is obtained, comprising paper folded in box shape carrying, interiorly only, a grease-resisting surface impregnum containing nitrocellulose and a grease-resisting resin.

It may be noted that I have employed a cottonseed phthalic glyceride resin in the

foregoing illustrations. This product is cheaply prepared from readily available materials, and has the advantage that cottonseed oil itself is employed as a softening material, hence the employment of cottonseed fatty acids in this manner does not introduce a foreign odor. Similarly fatty acids of other vegetable oils such as peanut oil, corn oil, soya bean oil, etc., may be incorporated in 10 resinous combination as described above. Castor oil may be used in some cases. The vegetable glycerides themselves may be resinated with phthalic anhydride or similar organic acid and glycol ethers. A striking feature of the glyceride and glycol resins and the like from the standpoint of the present invention is their repellent action on fatty oils. For example, the cottonseed phthalic glyceride, although containing in combination 20 the fatty acid components of cottonseed oil, is surprisingly resistant to animal and vegetable oils used in shortening, and this property enables the resin to serve to fortify and enhance any grease-proofing qualities which 25 nitrocellulose may possess.

The preferred coating or surfacing therefore consists of or contains nitrocellulose preferably of reduced viscosity, and a grease-repellent resin or balsam. The grease-repellent resins and balsams of the synthetic type may as aforesaid comprise a very large group of differing chemical and physical properties, but having in common the grease-repellent characteristic. This group 35 includes resins made from crystalline organic acids and their anhydrides, with such chemically different substances as glycols, chlorhydrines, glycol ethers, and glycerol, polyglycerol, and organic oxide such as ethylene or 40 butylene oxide.

Other solvent mixtures which may be used in the foregoing examples, or in modified compositions based on these illustrations, are: methyl acetate-benzol, ethyl acetate-denatured 45 alcohol, methyl acetate-denatured alcohol, isopropyl acetate-acetone, methyl acetone, ethyl-acetate-methyl alcohol, and so forth, these illustrations sufficing to indicate the various highly volatile solvents or mixed 50 solvents which may be employed.

In case there is desired a reduction in the combustibility of the nitrocellulose coating, tricresyl phosphate or triphenyl phosphate may be used for the purpose. It should be 55 noted, however, that the presence of the resin in the resinated nitrocellulose considerably reduces the rapidity of combustion of the latter, depending upon the proportion of resin present. Cellulose acetate may be used 60 to partly or wholly replace the nitrocellulose in cases where nitrocellulose is not desired.

As indicated above the ratio between nitrocellulose and resin may be varied considerably. This will depend to some extent upon 65 the character of the paper, on the flexibility

or pliability desired in the surfacing, on the length of time that the surface paper is likely to be kept before being cut and folded into cartons, as well as on other factors. A high proportion of nitrocellulose, that is, a major proportion, may be used in some cases, while in other cases the resin may predominate until ultimately a composition is reached where a small proportion of nitrocellulose merely serves to toughen a large proportion 70 of resin. The extremes on the one hand are represented by nitrocellulose alone, and on the other hand by the resin alone, and compositions made up with either of these extremes may be employed in some cases for 75 special purposes.

With respect to the additions of natural resins and the like, referred to above, a large proportion may easily impair the grease-repellent qualities of the synthetic resin, and any such dilution or cheapening of the resin by such additions should be avoided, since for best results I prefer not to use any resin 80 soluble in the common fatty oils employed as 85 shortening.

Preferably dye or coloring matter is not used in the resinated nitrocellulose solution, but the use of such coloring agents is not precluded, and if the exterior of the carton is 90 to be coated or surfaced with the resinated nitrocellulose sometimes it is desirable to employ a dye-stuff in the coating composition.

While the surfacing of resinated nitrocellulose increases water-resistance, I prefer to 100 employ, as I have indicated above, a board which has been made from paper pulp, to which a wax size, with or without a rosin size, has been incorporated prior to forming the pulp into sheets. By using such wax-containing 105 paper and supplementing the effect of the wax by the resinated nitrocellulose surfacing, I am able to obtain excellent water and grease resistance. This effect is improved by hot calendering.

When the board is used to make cartons it is desirable in some cases to pass it through hot rolls just before folding in order to render the coating more pliant. This is recommended particularly in cold weather.

In order to prevent diffusion of the vapors of the volatile solvents into the coating room, I may employ a small percentage of wax, such as paraffin or ceresine, in mixed solvents such as benzol-ethyl acetate. In my co-pending applications on the production of floor coverings by applying a surfacing containing nitrocellulose and resin, to a paper backing, (e. g. saturated felt) I have disclosed the employment of wax in amounts less than 1%. In the present invention I find it possible to somewhat increase the proportion of wax as blemishes which may be caused by the wax are largely removed on hot calendering. In 115 any event, however, I prefer not to use more 120

than 2 or 3% of wax, based on the weight of the solvent mixture used.

In using the term "resinated nitrocellulose" I do not, of course, mean to imply that the nitrocellulose itself is resinated, but that it is incorporated with a resin, particularly one compatible therewith.

In case the synthetic resins of the cotton-seed phthalic glyceride type are too soft, and it is desired to use only a low percentage of nitrocellulose, these resins may be increased in melting point by heating with one or two per cent or more of calcium hydrate, zinc hydrate or other hydrates, or oxides, or of a number of the metals. The resins of this type also may be rendered somewhat harder by treatment with sulphur chloride and careful removal of hydrochloric acid.

Referring again to the problem of producing an odorless surfacing, or one which does not emit any odor of a disagreeable character, or dissimilar to that of the foods contained in the carton, interiorly surfaced with the composition of the present invention, I wish to call attention to the fact that the employment of castor oil in the free state, blown castor oil, blown rapeseed oil, and the like, commonly used as softeners and plasticizers in nitrocellulose lacquers, is dangerous in the present case because the tendency of such oils to grow rancid and emit a disagreeable odor makes the employment of more suitable plasticizing agents desirable. The synthetic resins disclosed in the present invention, in which a fatty oil or fatty acid is in combination, preferably should be so made that the acid number is very low. The reaction in making the resin should be carried far enough to avoid high acid numbers. I prefer to employ resins with acid numbers below 20, or 30. Likewise in the case of nitrocellulose, I preferably avoid celluloid containing camphor because the latter gives a pronounced odor to food products. Furthermore, heavy solvents oftentimes employed as water eliminants in lacquers, leave a coating relatively slowly and may therefore generate an odor in the carton. By avoiding such heavy solvents, using highly volatile solvents instead, and employing a surfacing which substantially does not increase the thickness of the paper in order to permit of thorough evaporation of the solvent in the short space of time permissible for evaporation, the conditions are favored for production of a coating which does not generate an odor in the carton. If instead a heavy varnish-like surface were produced, a residual solvent may tend to create odors.

What I claim is:

1. Paper carrying nitrocellulose and a polybasic acid-polyhydric alcohol synthetic resin, the materials being present in an amount to give substantial grease repellent properties to the paper.

2. Wax-sized paper carrying nitrocellulose and polybasic acid-polyhydric alcohol synthetic resin, the materials being present in an amount to give substantial grease repellent properties to the paper. 70

3. Rosin-sized paper carrying nitrocellulose and polybasic acid-polyhydric alcohol synthetic resin, the materials being present in an amount to give substantial grease repellent properties to the paper. 75

4. Wrapping paper carrying a coating composition consisting essentially of nitrocellulose and polybasic acid-polyhydric alcohol synthetic resin, the materials being present in an amount to give substantial grease repellent properties to the paper and having been subjected to hot calendering subsequent to application. 80

5. A wrapping paper for grease containing articles, said paper carrying a coating of nitrocellulose and a polybasic acid-polyhydric alcohol synthetic resin, the materials being present in an amount to give substantial grease repellent properties to the paper. 85

6. A wrapping paper for grease containing articles, said paper carrying a coating of nitrocellulose and a polybasic acid-polyhydric alcohol synthetic resin, the materials being present in an amount to give substantial grease repellent properties to the paper, said paper having been subjected to hot calendering subsequent to the application of the coating. 90

7. A carton for containing greasy articles consisting of a paper coated with a material consisting essentially of nitrocellulose and polybasic acid-polyhydric alcohol synthetic resin, the materials being present in an amount sufficient to give substantial grease repellent properties to the paper. 100

8. A carton for containing greasy articles consisting of paper coated with a material consisting essentially of nitrocellulose and polybasic acid-polyhydric alcohol synthetic resin, the materials being present in an amount sufficient to give substantial grease repellent properties to the paper, said coating composition having been subjected to hot calendering subsequent to its application to the paper. 105

CARLETON ELLIS.

120

125

130